# EUROPEAN PATENT APPLICATION

(11) **EP 4 787 078 A1**
(43) Date of publication of application: **05.08.2026**
(21) Application number: 24871432.1
(22) Date of filing: 01.07.2024
(51) Int. Cl.: G03G 15/08, G03G 15/00

(54) **DEVELOPING ROLLER**

(30) Priority: 26.09.2023 JP 2023162233
(71) Applicant: Archem Inc., Tokyo 108-0075 (JP)
(72) Inventor: ISHIDA Ryo, Tokyo 108-0075 (JP)
(74) Representative: Scott, Stephen John
(86) International application number: PCT/JP2024/023844
(87) International publication number: WO 2025/069628

(57) **Abstract**

Provided is a development roller that can suppress toner leakage and fogging and that also excels in terms of stability of image density. The development roller includes a shaft member, an intermediate layer disposed radially outward of the shaft member, and a surface layer at an outermost position. The intermediate layer contains aggregates A formed of particles, dispersed in a resin. The surface layer contains granules B that are at least one selected from particles and aggregates formed of particles, dispersed in a resin. The granules B have an average diameter d_{B} of not less than 1 µm and not more than 10 µm.

## Description

### TECHNICAL FIELD

The present disclosure relates to a development roller.

### BACKGROUND

In electrophotographic image forming devices such as copiers and printers, a development method in which toner is supplied to a photosensitive drum bearing a latent image and in which the toner is caused to attach to the latent image of the photosensitive drum to cause visualization of the latent image is often adopted. Specifically, in this development method, development is performed by, for example, charging a photosensitive drum to a certain electrical potential, forming an electrostatic latent image on the photosensitive drum using an exposure tool, bringing a development roller bearing toner into contact with the photosensitive drum bearing the electrostatic latent image, and causing the toner to attach to the latent image on the photosensitive drum.

The development roller mentioned above typically has a structure in which an elastic layer that is formed of a semiconductive elastic body having a conductive agent dispersed in an elastomer such as polyurethane or a foam obtained through foaming of these materials is formed at the circumference of a shaft member that is installed with both longitudinal direction ends thereof axially supported. Moreover, there are instances in which a surface layer formed of a resin, etc. is formed at the outside of the elastic layer in the development roller described above with aims such as controlling charging and attachment properties with respect to toner, preventing fouling of a photosensitive drum, and so forth (for example, refer to Patent Literature (PTL) 1).

There are also instances in which fines particles are compounded in a layer (inclusive of the surface layer described above) that is disposed at the outside of the development roller in a radial direction in order to create unevenness. For example, PTL 2 discloses that toner supply capability is increased by providing one or more resin layers radially outward of a shaft member formed of a metal pipe and by dispersing fine particles in at least one of the resin layers so as to create surface roughness.

### CITATION LIST

### Patent Literature

PTL 1: JP 2005-352072 A
PTL 2: JP 2011-065188 A

### SUMMARY

### (Technical Problem)

When considering the surface roughness (unevenness) of a development roller, setting the protrusion height of the surface as at least a certain height makes it possible to suppress damage to a member (development blade, etc.) that comes into contact with the development roller and to suppress toner leakage from an end sealing member of an image forming device. The protrusion height of such a surface can be set at a high level by forming a layer in which fine particles having a comparatively large particle diameter are compounded.

However, when fine particles having a large particle diameter are used, it is difficult to uniformly disperse the fine particles in the layer, and uneven conveyance of toner and image fogging may arise during development.

In contrast, the use of fine particles having a comparatively small particle diameter enables uniform dispersion. However, the height (protrusion height) is insufficient in this case, meaning that suitable space cannot be provided between the surface of the development roller and a contacting member such as a development blade, and faults such as toner leakage can arise. In other words, toner leakage and fogging have an essentially antagonistic relationship.

Moreover, when the fine particles that are used are hard, the fine particles readily detach in that form in accompaniment to continuous or long-term operation of an image forming device, and there is a concern that variation of image density caused by significant changes of roughness will arise in such a situation.

Accordingly, the present disclosure addresses a problem of providing a development roller that can suppress toner leakage and fogging and that also excels in terms of stability of image density.

### (Solution to Problem)

Specifically, primary configurations of a development roller according to the present disclosure that solves the problem described above are as set forth below.
[1] A development roller comprising:
   a shaft member;
   an intermediate layer disposed radially outward of the shaft member; and
   a surface layer at an outermost position, wherein
   the intermediate layer contains aggregates A formed of particles, dispersed in a resin, and
   the surface layer contains granules B that are at least one selected from particles and aggregates formed of particles, dispersed in a resin, and the granules B have an average diameter d_{B} of not less than 1 µm and not more than 10 µm.
[2] The development roller according to [1], wherein the aggregates A in the intermediate layer have an average diameter d_{A} of not less than 10 µm and not more than 35 µm.
[3] The development roller according to [1] or [2], wherein content of the particles in the intermediate layer is not less than 10 parts by mass and not more than 30 parts by mass relative to 100 parts by mass of the resin.
[4] The development roller according to any one of [1] to [3], wherein content of the particles in the surface layer is not less than 15 parts by mass and not more than 35 parts by mass relative to 100 parts by mass of the resin.
[5] The development roller according to any one of [1] to [4], wherein the average diameter d_{A} of the aggregates A is larger than a thickness of the intermediate layer.
[6] The development roller according to any one of [1] to [5], wherein the average diameter d_{B} of the granules B is larger than a thickness of the surface layer.
[7] The development roller according to any one of [1] to [6], further comprising an elastic layer between the shaft member and the intermediate layer.
[8] The development roller according to any one of [1] to [7], further comprising an outer intermediate layer between the intermediate layer and the surface layer.

### (Advantageous Effect)

According to the present disclosure, it is possible to provide a development roller that can suppress toner leakage and fogging and that also excels in terms of stability of image density.

### BRIEF DESCRIPTION OF THE DRAWINGS

In the accompanying drawings:
FIG. 1 is a cross-sectional view of a development roller according to one embodiment of the present disclosure.

### DETAILED DESCRIPTION

### (Development roller)

The following provides a detailed illustrative description of a development roller according to the present disclosure based on embodiments thereof.

FIG. 1 is a cross-sectional view of a development roller according to one embodiment of the present disclosure (hereinafter, also referred to as the "development roller of the present embodiment"). A development roller 1 that is illustrated in FIG. 1 includes a shaft member 2, an elastic layer 3 disposed radially outward of the shaft member 2, an intermediate layer 4 disposed radially outward of the elastic layer 3, and a surface layer 5 disposed radially outward of the intermediate layer 4. It should be noted that the elastic layer 3 is not an essential configuration in the development roller according to the present disclosure. Also note that although the development roller 1 illustrated in FIG. 1 includes only one elastic layer 3, the development roller according to the present disclosure may include two or more elastic layers.

Features of the development roller 1 of the present embodiment are that the intermediate layer 4 contains aggregates A formed of particles, dispersed in a resin, the surface layer 5 contains granules B that are at least one selected from particles and aggregates formed of particles, dispersed in a resin, and the granules B have an average diameter d_{B} of not less than 1 µm and not more than 10 µm. Note that illustration of particles and aggregates is omitted in FIG. 1.

The intermediate layer 4 of the development roller 1 of the present embodiment has the aggregates A dispersed therein as described above. The aggregates referred to here normally have at least a certain size. Consequently, the aggregates A in the intermediate layer 4 bring about a suitable degree of unevenness (suitably high protrusions) at a circumferential surface of the development roller 1, thereby enabling suppression of toner leakage and also enabling suppression of damage to a member (development blade, etc.) that comes into contact with the development roller.

Moreover, by adopting aggregates as the dispersed media in the intermediate layer 4, this enables restriction to only partial shedding of the aggregates A, without overall detachment, even upon continuous or long-term operation of an image forming device that includes the development roller 1. Consequently, significant changes of surface roughness can be suppressed, and stability of image density can be maintained.

Furthermore, the surface layer 5 of the development roller 1 of the present embodiment has granules with a comparatively small particle diameter, and more specifically granules B having an average diameter d_{B} of 10 µm or less as described above, dispersed therein. Since the use of granules having a comparatively small particle diameter in this manner enables even more uniform dispersion, the provision of a layer containing the granules B described above as the surface layer can suppress image fogging during development.

Consequently, the development roller 1 of the present embodiment can suppress toner leakage and fogging and also excels in terms of stability of image density.

### <Shaft member>

The development roller 1 of the present embodiment includes a shaft member 2 as described above. The shaft member 2 is preferably a member having good conductivity. Specifically, the material of the shaft member 2 may be a metal such as iron, stainless steel, aluminum, or an alloy including any thereof, a plastic having good conductivity, or the like, for example. Moreover, the shaft member 2 may be a solid material or may be a hollow material (pipe). Furthermore, the shaft member 2 may include axle sections that constitute both longitudinal direction ends of the shaft member 2 such that the shaft member 2 is axially supported by roller supporting sections of an image forming device.

### <Intermediate layer>

The development roller 1 of the present embodiment includes an intermediate layer 4 disposed radially outward of the shaft member 2 as described above. The intermediate layer 4 contains aggregates A formed of particles, dispersed in a resin.

The constituent resin of the intermediate layer 4 may be a UV-curable resin, an electron beam-curable resin, or the like, for example, without any specific limitations. Specifically, the resin may be a polyester resin, polyether resin, fluororesin, epoxy resin, amino resin, polyamide resin, acrylic resin, acrylic urethane resin, urethane resin, alkyd resin, phenolic resin, melamine resin, urea resin, silicone resin, polyvinyl butyral resin, or the like. One of these resins may be used individually, or two or more of these resins may be used in combination. Of these resins, a UV-curable resin is preferable, and a urethane resin (UV-curable urethane resin) is more preferable as the constituent resin of the intermediate layer 4. Note that a urethane resin is formed through a reaction of a polyol component and a polyisocyanate component and has a property of undergoing curing through heat.

The intermediate layer 4 is required to have aggregates A formed of particles dispersed therein. In a case in which non-aggregates are used as the dispersed media, overall detachment of the non-aggregates arises upon continuous or long-term operation of an image forming device including the development roller 1, and stability of image density is poor.

The constituent particles of the aggregates A that are dispersed in the intermediate layer 4 may be particles of an organic material such as a silicone rubber, acrylic resin, styrene resin, acrylic/styrene copolymer, fluororesin (polytetrafluoroethylene (PTFE), etc.), urethane elastomer, urethane acrylate, melamine resin, or phenolic resin, for example, without any specific limitations. One of these types of particles may be used individually, or two or more of these types of particles may be used in combination. Of these examples, a fluororesin is preferable as the constituent particles of the aggregates A from a viewpoint of aggregability and ease of acquisition.

The deformation strength (σ_{10%}) of the constituent particles of the aggregates A that are dispersed in the intermediate layer 4 is preferably 1 MPa or less. When the deformation strength (σ_{10%}) of the particles is 1 MPa or less, damage to a photosensitive drum is suppressed, and fogging can be more effectively suppressed.

Note that the deformation strength (σ_{10%}) of the particles is the deformation strength at 10% compressive displacement of particle diameter and can be measured by a procedure described in the EXAMPLES section.

The average diameter d_{A} of the aggregates A dispersed in the intermediate layer 4 is preferably not less than 10 µm and not more than 35 µm. When the average diameter d_{A} is 10 µm or more, the effect of suppressing toner leakage can be further enhanced, and stability of image density can be maintained over a longer period. Moreover, when the average diameter d_{A} is 35 µm or less, image density unevenness can be suppressed, and the effect of suppressing fogging can be further enhanced. From similar viewpoints, the average diameter d_{A} of the aggregates A is more preferably 15 µm or more, and is more preferably 30 µm or less.

Note that the average diameter d_{A} of the aggregates A can be measured by a procedure described in the EXAMPLES section.

The average diameter d_{A} of the aggregates A dispersed in the intermediate layer 4 is preferably larger than the thickness (resin thickness) of the intermediate layer 4. In other words, when a resin composition containing the resin and the aggregates A is applied so as to form the intermediate layer 4, the resin composition is preferably applied with a thickness such that the aggregates A are partially protruding. This makes unevenness at the circumferential surface of the development roller 1 more noticeable and can more effectively suppress toner leakage. Note that the thickness (resin thickness) of the intermediate layer 4 can, in practice, be set as not less than 2 µm and not more than 10 µm, for example.

The diameter of the constituent particles of the aggregates A (i.e., the average primary particle diameter) is preferably not less than 0.1 µm and not more than 1 µm. When the average primary particle diameter is 0.1 µm or more, this facilitates gradual shedding of the aggregates A upon continuous or long-term operation of an image forming device including the development roller 1 and enables better maintenance of stability of image density. Moreover, when the average primary particle diameter is 1 µm or less, the desired aggregates A are easily formed.

The content of the particles in the intermediate layer 4 is preferably not less than 10 parts by mass and not more than 30 parts by mass relative to 100 parts by mass of the resin. When the content is 10 parts by mass or more, there is sufficiently high density of the aggregates A, and the effect of suppressing toner leakage can be further enhanced. Moreover, when the content is 30 parts by mass or less, coating non-uniformity during production of the intermediate layer 4 can be suppressed. From similar viewpoints, the content of the particles in the intermediate layer 4 is more preferably 15 parts by mass or more relative to 100 parts by mass of the resin, and is more preferably 25 parts by mass or less relative to 100 parts by mass of the resin.

Besides the resin and the aggregates A formed of particles, the intermediate layer 4 may contain other components such as a conductive agent.

### <Surface layer>

The development roller 1 of the present embodiment includes a surface layer 5 at an outermost position as described above. The surface layer 5 contains granules B that are at least one selected from particles and aggregates formed of particles, dispersed in a resin.

The constituent resin of the surface layer 5 is not specifically limited and may be any of those that were previously described as the constituent resin of the intermediate layer 4. One of these resins may be used individually, or two or more of these resins may be used in combination. Of these resins, a UV-curable resin is preferable, and a urethane resin (UV-curable urethane resin) is more preferable as the constituent resin of the surface layer 5. Note that the constituent resin of the surface layer 5 and the constituent resin of the intermediate layer 4 may be the same or different. However, it is preferable for the constituent resin of the surface layer 5 and the constituent resin of the intermediate layer 4 to be the same from a viewpoint of production efficiency.

The granules B dispersed in the surface layer 5 may be individual particles (non-aggregates), may be aggregates formed of particles, or may be both thereof.

The constituent particles of the granules B that are dispersed in the surface layer 5 are not specifically limited and may be any of those that were previously described as the constituent particles of the aggregates A that are dispersed in the intermediate layer 4. One of these types of particles may be used individually, or two or more of these types of particles may be used in combination. Of these types of particles, a fluororesin is preferable as the constituent particles of the granules B from a viewpoint of aggregability and ease of acquisition. Note that the constituent particles of the granules B and the constituent particles of the aggregates A may be the same or different. However, it is preferable for the constituent particles of the granules B and the constituent particles of the aggregates A to be the same from a viewpoint of production efficiency.

The average diameter d_{B} of the granules B dispersed in the surface layer 5 is required to be not less than 1 µm and not more than 10 µm. Note that the average diameter d_{B} of the granules B refers to the average primary particle diameter in a case in which the granules B are non-aggregates and refers to the average secondary particle diameter or aggregate diameter in a case in which the granules B are aggregates. In a situation in which the average diameter d_{B} of the granules B is less than 1 µm, the granules are too small, and it may not be possible to obtain the desired effect through compounding thereof. Moreover, in a situation in which the average diameter d_{B} of the granules B is more than 10 µm, it may not be possible to suppress fogging. Moreover, the average diameter d_{B} of the granules B is preferably 3 µm or more from a viewpoint of more reliably achieving the desired effect, and is preferably 8 µm or less from a viewpoint of more effectively suppressing fogging.

Note that the average diameter d_{B} of the granules B can be measured by a procedure described in the EXAMPLES section.

The average diameter d_{B} of the granules B is preferably smaller than the average diameter d_{A} of the aggregates A that are dispersed in the intermediate layer 4. In other words, a ratio of the average diameter d_{B} of the granules B relative to the average diameter d_{A} of the aggregates A (average diameter d_{B}/average diameter d_{A}) is preferably less than 1.0. With regards to this point, the granules B can easily be obtained through micronization of the aggregates A using a dispersant or the like in a case in which the constituent particles of the granules B and the constituent particles of the aggregates A are the same type of particles. Moreover, the aforementioned ratio (average diameter d_{B}/average diameter d_{A}) is more preferably 0.7 or less, and even more preferably 0.4 or less.

The average diameter d_{B} of the granules B dispersed in the surface layer 5 is preferably larger than the thickness (resin thickness) of the surface layer 5. In other words, when a resin composition containing the resin and the granules B is applied so as to form the surface layer 5, the resin composition is preferably applied with a thickness such that the granules B are partially protruding. This makes unevenness at the circumferential surface of the development roller 1 more noticeable and can more effectively suppress toner leakage. Note that the thickness (resin thickness) of the surface layer 5 can, in practice, be set as not less than 1 µm and not more than 5 µm, for example. Moreover, the thickness (resin thickness) of the surface layer 5 may be smaller than the thickness (resin thickness) of the intermediate layer 4.

The content of the particles in the surface layer 5 is preferably not less than 15 parts by mass and not more than 35 parts by mass relative to 100 parts by mass of the resin. When the content is 15 parts by mass or more, there is sufficiently high density of the granules B, and effects such as improving toner supply capability are achieved. Moreover, when the content is 35 parts by mass or less, coating non-uniformity during production of the surface layer 5 can be suppressed, and the effect of suppressing fogging can be further enhanced. From similar viewpoints, the content of the particles in the surface layer 5 is more preferably 20 parts by mass or more relative to 100 parts by mass of the resin, and is more preferably 30 parts by mass or less relative to 100 parts by mass of the resin.

Besides the resin and the granules B, the surface layer 5 may contain other components such as a conductive agent.

### <Elastic layer>

The development roller 1 of the present embodiment preferably further includes an elastic layer 3 between the shaft member 2 and the intermediate layer 4 as illustrated in FIG. 1. This makes it possible to impart elasticity to the development roller 1 and relieve stress acting on the surface layer 5 when the surface layer 5 of the development roller 1 is pressed against a photosensitive drum or a development blade, and also enables good maintenance of durability of the surface layer 5.

The elastic layer 3 is preferably formed of an elastomer, and is more preferably formed of a foam of an elastomer. The elastomer may be a polyurethane, silicone rubber, ethylene-propylene-diene rubber (EPDM), acrylonitrile-butadiene rubber (NBR), natural rubber (NR), styrene-butadiene rubber (SBR), butadiene rubber (BR), isoprene rubber (IR), polynorbornene rubber, butyl rubber (IIR), chloroprene rubber (CR), acrylic rubber, epichlorohydrin rubber (ECO), ethylene-vinyl acetate copolymer (EVA), or the like, for example. One of these elastomers may be used individually, or two or more of these elastomers may be used in combination. In particular, of these elastomers, a polyurethane is preferably used in the elastic layer 3.

The foam of the elastomer can be produced by using a foaming agent to perform chemical foaming of the elastomer or by mechanically incorporating air to cause foaming such as in polyurethane foam. In a case in which the elastic layer 3 is formed from a foam of an elastomer, the foam preferably has a foam expansion ratio in a range of ×1.5 to ×50, and preferably has a density in a range of 0.05 g/cm³ to 0.9 g/cm³.

Moreover, cells in the foam described above are preferably closed cells. In this case, compression set performance of the elastic layer 3 can be improved. The method by which cells of the foam are formed as closed cells may suitably be a method in which a raw material of the elastomer is foamed through mechanical stirring to obtain the foam.

The elastic layer 3 preferably contains a conductive agent. This makes it possible to adjust conductivity of the elastic layer 3. The conductive agent may be an electronic conductive agent, an ionic conductive agent, or the like. One conductive agent may be used individually, or two or more conductive agents may be used in combination. Moreover, an electronic conductive agent and an ionic conductive agent may be used in combination as the conductive agent.

Examples of the electronic conductive agent include conductive carbon such as Ketjen Black and acetylene black, carbon black for rubber such as SAF, ISAF, HAF, FEF, GPF, SRF, FT, and MT, carbon black for coloring that has been subjected to oxidation treatment or the like, pyrolyzed carbon black, natural graphite, artificial graphite, metal oxides such as antimony-doped tin oxide, ITO, tin oxide, titanium oxide, and zinc oxide, metals such as nickel, copper, silver, and germanium, conductive polymers such as polyaniline, polypyrrole, and polyacetylene, and conductive whiskers such as carbon whiskers, graphite whiskers, titanium carbide whiskers, conductive potassium titanate whiskers, conductive barium titanate whiskers, conductive titanium oxide whiskers, and conductive zinc oxide whiskers.

Examples of the ionic conductive agent include ammonium salts such as perchlorates, chlorates, hydrochlorides, bromates, iodates, hydrofluoroborates, sulfates, ethyl sulfates, carbonates, and sulfonates of tetraethylammonium, tetrabutylammonium, dodecyltrimethylammonium, hexadecyltrimethylammonium, benzyltrimethylammonium, and modified fatty acid dimethylethylammonium; and perchlorates, chlorates, hydrochlorides, bromates, iodates, hydrofluoroborates, sulfates, trifluoromethyl sulfates, and sulfonates of alkali metals and alkaline earth metals such as lithium, sodium, potassium, calcium, and magnesium.

### <Other layers>

The development roller 1 of the present embodiment can further include layers other than the intermediate layer 4, the surface layer 5, and the elastic layer 3 described above.

For example, the development roller 1 of the present embodiment may further include an outer intermediate layer (not illustrated) radially outward of the intermediate layer 4, and, more specifically, between the intermediate layer 4 and the surface layer 5. The outer intermediate layer may be a single layer or may be two or more layers. This outer intermediate layer can function as an adhesive layer, and the inclusion of the outer intermediate layer can increase adhesiveness between the intermediate layer 4 and the surface layer 5 and increase durability of the development roller 1.

No specific limitations are placed on a constituent resin of the outer intermediate layer, and any of those that were previously described as the constituent resin of the intermediate layer 4 may be used. One of these resins may be used individually, or two or more of these resins may be used in combination. The thickness (per one layer) of the outer intermediate layer can be set as not less than 1 µm and not more than 5 µm, for example.

The development roller 1 of the present embodiment can further include an inner intermediate layer (not illustrated) radially inward of the intermediate layer 4, and, more specifically, between the intermediate layer 4 and the shaft member 2 or the elastic layer 3. The inner intermediate layer may be a single layer or may be two or more layers. This inner intermediate layer can function as an adhesive layer, and the inclusion of the inner intermediate layer can increase adhesiveness between the intermediate layer 4 and the shaft member 2 or the elastic layer 3 and can increase durability of the development roller 1.

No specific limitations are placed on a constituent resin of the inner intermediate layer, and any of those that were previously described as the constituent resin of the intermediate layer 4 may be used. One of these resins may be used individually, or two or more of these resins may be used in combination. The thickness (per one layer) of the inner intermediate layer can be set as not less than 1 µm and not more than 5 µm, for example.

### <Production method of development roller>

The development roller of the present embodiment can be produced according to a standard method without any specific limitations on the production method. For example, each of the layers such as the intermediate layer 4 and the surface layer 5 can be formed by preparing a resin composition (coating liquid) containing a resin, particles and/or aggregates, and other components as appropriate, applying the coating liquid onto a surface, and then optionally irradiating the coating liquid with ultraviolet radiation or an electron beam to cure the coating liquid.

The method by which the resin composition (coating liquid) is applied may be dip coating, roll coating, spray coating, or the like without any specific limitations and can be selected as appropriate from these methods according to the circumstances.

### <Application of development roller>

The development roller according to the present disclosure can be used in various types of electrophotographic image forming devices such as copiers, fax machines, and laser beam printers (LBPs). The image forming device normally includes a photosensitive drum that bears an electrostatic latent image, a charging member that is located in proximity to the photosensitive drum and that charges the photosensitive drum, a toner supply roller for supplying toner, a transfer member that is located in proximity to the photosensitive drum, and a cleaning member that is located adjacently to the photosensitive drum, and further includes the development roller between the toner supply roller and the photosensitive drum. In addition, a development blade (also referred to as a "layering blade") is normally provided in proximity to the development roller.

In the image forming device, voltage is applied between the photosensitive drum and the charging member so as to charge the photosensitive drum to a certain electrical potential, and then an electrostatic latent image is formed on the photosensitive drum using an exposure tool. Next, toner is fed from the toner supply roller to the photosensitive drum via the development roller. During this feeding, toner on the development roller is leveled into a more uniform thin layer by the development blade, and the development roller and the photosensitive drum rotate while coming into contact to thereby cause the toner to attach onto the electrostatic latent image of the photosensitive drum from the development roller and cause visualization of the latent image. Toner that has become attached to the latent image is transferred to a recording medium such as paper by the transfer member, and toner that remains on the photosensitive drum after transfer is removed by the cleaning member.

As a result of the development roller according to the present disclosure being used in the image forming device, toner leakage and fogging can be suppressed. Moreover, stability of image density can be maintained even upon continuous or long-term operation this image forming device.

### EXAMPLES

The following provides an even more detailed description of the present disclosure through examples. However, the present disclosure is not in any way limited by these examples, and changes can be made as appropriate to the extent that the essence of the present disclosure is not changed.

### (Example 1)

An elastic layer, an intermediate layer, an outer intermediate layer (adhesive layer), and a surface layer were formed in this order on a shaft member formed of an aluminum pipe to thereby produce a development roller. Note that the intermediate layer was formed by applying, onto the elastic layer by roll coating, a resin composition obtained by compounding aggregates of polytetrafluoroethylene particles in a urethane resin (main conditions of the intermediate layer are as indicated in Table 1). The adhesive layer was formed by applying a resin composition (coating liquid, purchased product) onto the intermediate layer by roll coating. The surface layer was formed by spraying, onto the adhesive layer by spray coating, a resin composition (dispersion liquid) obtained by compounding aggregates of polytetrafluoroethylene particles in a solvent containing a urethane resin (main conditions of the surface layer are as indicated in Table 1).

Note that in Example 1, the same particles were used as constituent particles of aggregates in the intermediate layer and constituent particles of aggregates in the surface layer and that the aggregates in the surface layer had undergone further micronization using a dispersant or the like than the aggregates in the intermediate layer.

The average diameter d_{A} of aggregates A (or particles) dispersed in the intermediate layer was measured by the following procedure.

Specifically, after formation of the intermediate layer, a laser microscope (VK-X3000 produced by Keyence Corporation) was used to acquire a surface image of a longitudinal direction central section of the intermediate layer. Next, 100 aggregates A (or particles) were counted in this surface image, and outer diameter data of these 100 aggregates A was acquired. The outer diameter data was used to calculate D50 as the average diameter d_{A}.

The average diameter d_{B} of granules B dispersed in the surface layer was measured by the following procedure.

Specifically, after formation of the surface layer, a laser microscope (VK-X3000 produced by Keyence Corporation) was used to acquire a surface image of a longitudinal direction central section of the surface layer. Next, 100 granules B were counted in this surface image, and outer diameter data of these 100 granules B was acquired. The outer diameter data was used to calculate D50 as the average diameter d_{B}.

The deformation strength (σ_{10%}) of particles was measured by the following procedure.

Specifically, a microparticle compression strength tester (NS-A100 produced by Nano Seeds Corporation) was used to determine the deformation strength (σ_{10%}) by the following formula.${σ}_{10 %} = {F}_{10 %} / A$
σ_{10%}: Deformation strength (Pa) at 10% compressive displacement of particle diameter
F_{10%}: Test force (N) at 10% compressive displacement of particle diameter
A: Representative area (area of equivalent circle determined through particle diameter of particle measured before compression) (m²)

### (Other examples and comparative examples)

Development rollers were produced in the same way as in Example 1 with the exception that conditions of the intermediate layer and/or the surface layer were changed as indicated in Table 1.

The development roller of each example or comparative example that had been produced as described above was subjected to the following evaluations. The results are shown in Table 1.

### (1) Initial image density

The produced development roller was installed in a monochrome laser printer "HL-L6400DW" produced by Brother, and a solid black image was printed. A spectrodensitometer "eXact Basic" produced by X-Rite, Incorporated was used to measure image density at 5 locations on the paper surface for the obtained image. An average value (average density) and the difference between maximum and minimum values (density difference) were calculated for the densities at the 5 locations and were evaluated by the following standard.
A (Very good): Average density of 1.2 or more and density difference of 0.2 or less
B (Good): Average density of 1.2 or more and density difference of less than 0.2
C (Poor): Average density of less than 1.2

### (2) Image density after endurance printing (stability of image density)

After measurement of the initial image density as described above, endurance printing (printing of approximately 20,000 sheets of solid black images) was performed. A spectrodensitometer "eXact Basic" produced by X-Rite, Incorporated was used to measure image density at 5 locations on the paper surface for a final image that was obtained. An average value (average density) and the difference between maximum and minimum values (density difference) were calculated for the densities at the 5 locations and were evaluated by the following standard.
A (Very good): Average density of 1.2 or more and density difference of 0.2 or less
B (Good): Average density of 1.2 or more and density difference of less than 0.2
C (Poor): Average density of less than 1.2

### (3) Fogging

The produced development roller was installed in a monochrome laser printer "HL-L6400DW" produced by Brother, and a durability test was performed in an LL environment (10°C, 15%RH). An image obtained after the test was evaluated by the following standard.
A (Very good): Fixing of toner not observed at locations in image where toner should not be present
B (Good): Slight fixing of toner observed at locations in image where toner should not be present
C (Poor): Widespread fixing of toner observed at locations where toner should not be present

### (4) Toner leakage

The produced development roller was installed in a monochrome laser printer "HL-L6400DW" produced by Brother, and durability tests were performed in an LL environment (10°C, 15%RH) and an HH environment (30°C, 80%RH). Thereafter, the condition of toner around the development roller was evaluated by the following standard.
A (Very good): Spraying of toner from ends of development roller and seal fouling not observed
B (Good): Spraying of toner from ends of development roller not observed, but seal fouling observed
C (Poor): Spraying of toner from ends of development roller and seal fouling both observed

### [Table 1]

**Table 1**

| | | | Example 1 | Comparative Example 1 | Comparative Example 2 | Example 2 | Example 3 | Comparative Example 3 | Example 4 | Example 5 |
|---|---|---|---|---|---|---|---|---|---|---|
| Surface layer | Particles | Material | PTFE | PTFE | PTFE | PTFE | PTFE | PTFE | PTFE | PTFE |
| | | Aggregation | Yes | Yes | Yes | Yes | Yes | Yes | Yes | Yes |
| | | Average diameter d_{B} [µm] | 3 | 3 | 3 | 1 | 8 | 15 | 4 | 4 |
| | | Average primary particle diameter [µm] | 0.2 | 0.2 | 0.2 | 0.2 | 0.2 | 0.2 | 0.2 | 0.2 |
| | | Deformation strength σ10% [MPa] | 0.5 | 0.5 | 0.5 | 0.5 | 0.5 | 0.5 | 0.5 | 0.5 |
| | | Content [parts by mass/100 parts by mass of resin] | 20 | 33 | 20 | 20 | 20 | 20 | 20 | 20 |
| | Thickness [µm] | | 2 | 2 | 2 | 2 | 2 | 2 | 2 | 2 |
| Intermediate layer | Particles | Material | PTFE | - | Acrylic resin | PTFE | PTFE | PTFE | PTFE | PTFE |
| | | Aggregation | Yes | | No | Yes | Yes | Yes | Yes | Yes |
| | | Average diameter d_{A} [µm] | 15 | | 30 | 20 | 20 | 15 | 5 | 40 |
| | | Average primary particle diameter [µm] | 0.2 | | | 0.2 | 0.2 | 0.2 | 0.2 | 0.2 |
| | | Deformation strength σ10% [MPa] | 0.5 | | 30 | 0.5 | 0.5 | 0.5 | 0.5 | 0.5 |
| | | Content [parts by mass/ 100 parts by mass of resin] | 20 | 0 | 20 | 20 | 20 | 20 | 20 | 20 |
| | Thickness [µm] | | 2 | 2 | 2 | 2 | 2 | 2 | 2 | 2 |
| Evaluation | Initial image density | | A | A | A | A | A | B | A | B |
| | Image density after endurance printing | | A | A | C | A | A | B | A | B |
| | Fogging | | A | A | C | A | A | C | A | B |
| | Toner leakage | | A | C | A | B | A | A | B | A |

It can be seen from Table 1 that the development rollers of the examples in accordance with the present disclosure can suppress toner leakage and fogging and also excel in terms of stability of image density.

### INDUSTRIAL APPLICABILITY

The development roller according to the present disclosure can be used in various electrophotographic image forming devices such as copiers, fax machines, and laser beam printers (LBPs).

### REFERENCE SIGNS LIST

- 1: development roller
- 2: shaft member
- 3: elastic layer
- 4: intermediate layer
- 5: surface layer

## Claims

1. A development roller comprising:
a shaft member;
an intermediate layer disposed radially outward of the shaft member; and
a surface layer at an outermost position, wherein
the intermediate layer contains aggregates A formed of particles, dispersed in a resin, and
the surface layer contains granules B that are at least one selected from particles and aggregates formed of particles, dispersed in a resin, and the granules B have an average diameter d_{B} of not less than 1 µm and not more than 10 µm.

2. The development roller according to claim 1, wherein the aggregates A in the intermediate layer have an average diameter d_{A} of not less than 10 µm and not more than 35 µm.

3. The development roller according to claim 1 or 2, wherein content of the particles in the intermediate layer is not less than 10 parts by mass and not more than 30 parts by mass relative to 100 parts by mass of the resin.

4. The development roller according to claim 1 or 2, wherein content of the particles in the surface layer is not less than 15 parts by mass and not more than 35 parts by mass relative to 100 parts by mass of the resin.

5. The development roller according to claim 1 or 2, wherein the average diameter d_{A} of the aggregates A is larger than a thickness of the intermediate layer.

6. The development roller according to claim 1 or 2, wherein the average diameter d_{B} of the granules B is larger than a thickness of the surface layer.

7. The development roller according to claim 1 or 2, further comprising an elastic layer between the shaft member and the intermediate layer.

8. The development roller according to claim 1 or 2, further comprising an outer intermediate layer between the intermediate layer and the surface layer.
